

March 31, 1925.

1,531,827

J. C. ARMOR

FILLER ROD FOR FUSION WELDING

Filed Dec. 6, 1922



WITNESS  
R.F. Dilworth

INVENTOR.  
James C. Armor,  
BY Edward A. Lawrence,  
his ATTORNEYS.

Patented Mar. 31, 1925.

1,531,827

# UNITED STATES PATENT OFFICE.

JAMES C. ARMOR, OF WEST VIEW BOROUGH, PENNSYLVANIA.

## FILLER ROD FOR FUSION WELDING.

Application filed December 6, 1922. Serial No. 605,305.

*To all whom it may concern:*

Be it known that I, JAMES C. ARMOR, a citizen of the United States, and residing in the borough of West View, in the county 5 of Allegheny and State of Pennsylvania, have invented or discovered the new, useful, and Improved Filler Rod for Fusion Welding, of which the following is a specification.

My invention consists in a new and improved 10 filler rod for use in connection with the same.

In joining metals together by fusion welding, it is evident that no given composition 15 filler rod will produce equally good results with all metals, or even when using the same metal for all classes of work.

Thus, in mild steel, great tensile strength 20 may be required in one class of work, in another great hardness; in another ductility and softness, etc.

To obtain the various characteristics required, it is necessary to vary the composition of the metal or to use alloys.

However, it is very difficult and very 25 expensive to produce filler rods of certain compositions of metals and certain alloys, and in many cases the filler rods, when heated, rapidly oxidized and deteriorate. Another difficulty is that certain of the compositions 30 and alloys melt at too low temperatures and others form very large drops, thus preventing the formation of a perfect weld.

For these, and other reasons, it has been 35 found impractical in the past to use many compositions and alloys in fusion welding, although such compositions and alloys are best fitted for the purposes in view.

To overcome these and other difficulties, I 40 abandon the previous practice of attempting to combine the elements in the form of a composition or alloy in the filler rod, but unite the elements at the point of fusion at the weld.

For convenience and to enable me to properly 45 associate the elements in proper juxtaposition at the weld, I mechanically associate the elements together in the filler rod.

Thus in my improved filler rod, all of the 50 elements of the desired composition or alloy are mechanically associated together in the rod, but are not actually combined until they are melted and deposited in the weld.

Thus as a preferred form of my invention, I 55 use a filler rod consisting of a tube or cylinder of one metal surrounding a core composed of the other metal or metals or an

alloy of the same. Where a plurality of metals or elements are used I may form the outer tube or the core of two or more elements which may be advantageously combined before being applied to the weld. I also prefer to mix or associate with the material of the core, or if desired, with the material of the outer tube a suitable flux or flux-forming substance or substances, and also, 65 where advantageous, suitable reducing and scavenging elements.

For instance, where nickel steel is required, I may make the outer tube of steel, while the core contains the desired amount 70 of nickel, either as a powder or in the form of a wire, the nickel being in either case combined or associated with a suitable flux.

Again if bronze be required, the tube may be of copper and the core may contain tin 75 and other desired elements together with a suitable flux.

I may form the filler rod by using a wire 80 of grooved or U-shaped cross section composed of the metal or metals, which are to form the outer tube, then introduce the element or elements, which are to form the core, in the form of powder into the groove, the walls of the groove being then closed together to inclose the core.

Thus in Fig. 1 of the accompanying drawings, I show in perspective a length of said wire A into whose longitudinal groove is introduced the core material B, and the walls of the groove are then brought together to 90 form a tube 'A' in closing the core material B'.

In Fig. 2 I show in perspective, a filler rod composed of an outer tube C composed of one or more of the elements, and having its axial bore occupied by a wire D composed of the remaining elements.

It is evident from the foregoing that my improved filler rod enables me to unite and combine the elements when melted in the weld, and thus avoid the difficulties above mentioned and which have attended the attempts to form a filler rod of the elements in composition or alloy.

If desired my filler rod may be used in the manufacture of desired alloys by merely melting the rod in a suitable crucible or mold.

What I desire to claim is:—

1. A filler rod for use in fusion welding consisting of an outer inclosing wall formed of one or more elements of a com-

- position metal or alloy, and a central core formed of the remaining element or elements together with a suitable flux.
2. A filler rod for use in fusion welding comprising an enclosed outer wall formed of one or more of the elements of a composition metal or alloy, and a central core, enclosed by said outer wall and comprising a mixture of flux and materials, in powdered form adapted to react with or be added to the metal of the outer wall after the same has passed through the arc.
3. A filler rod for use in fusion welding consisting of an outer sheath formed of one or more of the elements of the composition metal or alloy, and enclosed therein a core comprising a mixture of powdered flux and materials which combine after passage through the arc with the material of the outer sheath to form an alloy of the desired characteristic.

Signed at Pittsburgh, Pa., this 2nd day of December, 1922.

JAMES C. ARMOR.